

S. E. SHEPPARD.

COLORED PHOTOGRAPHIC ELEMENT AND PROCESS OF MAKING THE SAME.

APPLICATION FILED MAY 24, 1917.

1,290,794.

Patented Jan. 7, 1919.

FIG. 1.



FIG. 2.



FIG. 3.



FIG. 4.



FIG. 5.



FIG. 6.



WITNESSES:

*Frederick Stewart*  
Newton M. Dennis

INVENTOR.  
*Samuel E. Sheppard*,  
BY *R. L. Stinchfield*

ATTORNEY

# UNITED STATES PATENT OFFICE.

SAMUEL E. SHEPPARD, OF ROCHESTER, NEW YORK, ASSIGNOR TO EASTMAN KODAK COMPANY, OF ROCHESTER, NEW YORK, A CORPORATION OF NEW YORK.

## COLORED PHOTOGRAPHIC ELEMENT AND PROCESS OF MAKING THE SAME.

1,290,794.

Specification of Letters Patent.

Patented Jan. 7, 1919.

Application filed May 24, 1917. Serial No. 170,777.

*To all whom it may concern:*

Be it known that I, SAMUEL E. SHEPPARD, a subject of the King of Great Britain, and a resident of Rochester, county of Monroe, 5 and State of New York, have invented certain new and useful Improvements in Colored Photographic Elements and Processes of Making the Same, of which the following is a specification.

0 My invention relates to colored elements for photographic purposes and processes of making the same, and more particularly to a translucent colored, finely divided or colloidal substance in a supporting medium 5 capable of use on a photographic element or with photographically sensitive material in the art of photography. An object of my invention is to provide a colored medium for use on a photographic plate, containing 0 water fast colored particles which will not bleed or migrate from their carrier into adjacent materials during treatment thereof in the usual photographic baths and furthermore to furnish a preferably translucent medium which is capable of being coated on a surface like a photographic emulsion and of being used as or mixed with photographic material for use on a plate, film, paper, or other surface. With these and other objects in view, as will appear hereinafter from the following disclosure, my invention consists in the combination of parts and the steps of processes described in the specification and covered by the claims annexed hereto.

In accordance with my discoveries, I have found it desirable to provide a colored medium for various photographic uses and especially to incorporate a dye or other color material in a medium capable of being coated photographically. Gelatin is ordinarily used for photographic coating purposes, but it is found, however, that if gelatin is dyed, there is a tendency for desirable types of dye to bleed or run, or to wander from the gelatin into aqueous solutions, so that the color is either discharged or is not permanently located and the colored mass is not well adapted for photographic, photomechanical or other purposes, since photographic intensity and definition are affected by the wandering of the dye. On the other hand cellulose compounds, such as nitrocellulose, cellulose acetate, etc., tend to hold basic dyes in molecular or a fixed relation thereto, and on this fact my discoveries are based. If nitro-

cellulose is placed in an aqueous gelatin solution containing a basic dye, the color tends to wander from the gelatin to the nitrocellulose and to fix itself in the latter. Furthermore, the dyes usually employed to dye gelatin are acid dyes, which are unsuitable for use on photographic plates, since the ordinary developer, having an alkaline reaction, tends to affect the dye chemically. It has also been found that basic or neutral dyes 60 do not ordinarily dye gelatin fast, except in the form of a precipitated dye lake obtained by the action of a mordant upon a dye, and such lakes have a tendency to sadden the colors and to affect the photographic properties of the gelatin.

In accordance with my invention, I utilize as a dye carrying medium cellulose compounds such as cellulose acetates, nitrates, ethers, esters, etc., with or without, as may 75 be necessary, such latent solvents as camphor, etc., and color the same by means of basic dyes, thus obviating the many disadvantages arising from dyeing gelatin, due to the presence of other substances such as 80 alkali, or the difficulties of obtaining sharp photographic images arising from a wandering of the dye. I find it desirable to utilize a colloid, such as gelatin, as a basis for my colored medium, hence I mix therewith my 85 color bearing elements. It is not feasible to incorporate a pigment in the gelatin for many reasons, including the facts that the pigment particles are of relatively large size and are opaque and reflecting and not sufficiently transparent to actinic light rays; but it is highly desirable that the dye carrier involve material having such properties that light may pass readily through it.

I have found that nitrocellulose and similar compounds, besides being excellent dye carriers and translucent to actinic light, are capable of being emulsified or transformed into a state of fine suspension, so that when mixed with a supporting mass, such as gelatin, there is formed a color medium which is practically homogeneous to the eye and which allows a substantially uniform passage throughout its mass of light colored according to the transmission of the dye, 105 Colloidal materials are ideal for photographic emulsions, and I find it desirable to use such agglutinating colloids as gelatin, agar-agar, fish glue or water soluble colloids as the magma or holder of my colored par- 110

ticles. In order that the mixture may be uniform in composition, I find it desirable to finely divide or emulsify a mass of dyed cellulose compound in the colloid, such as 5 an aqueous solution of gelatin, and thereby obtain an emulsion, similar to a photographic emulsion of silver bromid in gelatin, which may be coated or otherwise employed.

- 10 If nitrocellulose is selected for the color medium, I may dissolve it in a suitable solvent such as amyl acetate and color the nitrocellulose either before or after by adding a dye thereto, depending on the nature of 15 the latter. The nitrocellulose is then transformed from its dissolved state into one of a fine suspension or emulsion and incorporated with a colloidal or gelatinous carrier, while the dye remains wash fast in the nitrocellulose and does not leave it during the 20 intermediate chemical or physical changes. This step of incorporating one material with the other is accomplished preferably by the aid of an emulgent and stirring operations, 25 after which the colloidal mass or emulsion thus formed may be suitably purified or otherwise prepared for use. I thereby form an emulsion or suspension of more or less fine particles of partially gelatinized dyed 30 nitrocellulose in a carrier, such as gelatin.

#### *Dyeing the nitrocellulose.*

In order to obtain dyed nitrocellulose, it is necessary to proceed in the manner indicated by the nature of the dye desired to be employed. Some dyes should be added to the nitrocellulose before it is dissolved in amyl acetate while others may be added to the acetate solution.

- 40 The dye which may be added to the cellulose derivative either before or after it is dissolved in the acetate, may comprise a basic dye or dyestuff soluble in oil, spirit, or both, and insoluble in water. For example, one may utilize the group of so called 45 oil soluble dyestuffs comprising such dyes as Soudan dyes, *e. g.*, spirit soluble red O. G. as a red dye, or such dyes as malachite green, a green dye. If the dyestuff is oil soluble 50 it may be directly dissolved in the amyl acetate solution of nitrocellulose; for example, a dye such as red O. G. is soluble in amyl acetate. Otherwise it is advisable 55 that the dye be first dissolved, in a small quantity of alcohol, which may be mixed with the nitrocellulose solution in amyl acetate.

Various methods of converting water soluble dyes into spirit soluble dyes may be 60 employed depending on the chemical characteristics of the dye materials. For example, one may use a basic dye, which is insoluble in alcohol and soluble in water, but which forms a tannate with tannic acid, if 65 the tannate is soluble in alcohol and insoluble

in water. In case the use of a tannate is adopted the tendency of the gelatin to be tanned or insolubilized may be avoided by treating the tannate with tartar emetic or potassium antimony tartrate or other soluble 70 antimony salts.

If an alcohol soluble dye, or an alcohol soluble compound thereof, such as a tannate, is used, I find it feasible to dissolve the same in alcohol and preferably a mixture of 75 ethyl and methyl alcohol, of which the ethyl alcohol may be 95% alcohol. In other words, absolute alcohol need not be used. I incorporate this alcohol solution with the acetate solution. The greater portion of the 80 alcohol may be then distilled off, leaving the acetate behind.

If the so called hard nitrocellulose is employed as the dye carrier, it is quite feasible to dissolve it in acetone, or acetone and 85 methyl alcohol, and then add the dyestuff thereto to color the material. Upon throwing this colored mass into hot water or otherwise treating it with hot water, the dyed nitrocellulose is precipitated out, and 90 all dye in excess stays in the acetone solution, provided an excess of acetone-alcohol and not too large an amount of dye is used. The precipitated dyed nitrocellulose may then be dried for subsequent treatment. 95

#### *Dissolving the dyed nitrocellulose.*

In order to dissolve dyed nitrocellulose, which may be obtained by the above described methods, it is desirable for the purposes of my invention to employ a substance which forms a solution capable of being emulsified. Furthermore, the solvent should be normally insoluble in the water in which the gelatin is dissolved and normally indifferent to gelatin so as not to precipitate the latter from its solution. For this purpose amyl acetate is highly suitable, and the step may be carried out according to well known chemical operations. 100

By these or other methods serving to accomplish the same general result, I obtain a solution of a cellulose compound, as nitrocellulose, in a solvent such as amyl acetate, in which a suitable dye is incorporated. The dye is thereby fixed in a carrier which is capable of being finely divided into a more or less homogeneous mass without losing its color characteristics imparted to it by the dye. 11

#### *Emulsifying the dyed solution.*

In order to make an emulsion, suspension or a colloidal mass from this dyed compound, the amyl acetate solution of nitrocellulose is introduced into or incorporated with a solution of gelatin in such a manner that the nitrocellulose assumes a finely divided or colloidal condition and remains suspended in or mixed with the gelatin 1

which serves as a carrier for the dyed particles.

To facilitate the operation of emulsifying or transforming the nitrocellulose into a 5 colloidal condition, the use of a suitable emulgent is desirable. For this purpose I prefer to employ Turkey red oil, *i. e.*, sulfonated castor oil, and may adopt any well known method of producing the emulsion. 10 For example, the solution of dyed nitrocellulose may be introduced, as by an atomizer, in a state of fine subdivision into the gelatin solution and the mass agitated until the emulsion has been formed, the solution being 15 kept liquid by maintaining the temperature above the setting point of the gelatin. Regulation of the temperature controls the viscosity of the solution and thereby is of marked importance in determining the size 20 of particles to be obtained. If desired, the emulsion may be homogenized in its present oily stage, in order to obtain colloidal particles of uniform size, this operation being carried out by any suitable well known 25 means. For example, one may throw the emulsion against baffle plates by centrifugal force, thus causing the particles to assume sizes that are more or less of the same order of magnitude.

30 As a specific example of the above steps of my process, I may take 3 grams of the solid dyestuff, spirit soluble red O. G., and dissolve this in a solution of 5 grams of hard nitro cotton in 100 cc. of amyl acetate. This 35 solution is introduced slowly from below into 500 cc. of 10% solution of gelatin in water containing 5 cc. of Turkey red oil, the solution being kept liquid at from 50° C. to 60° C.

#### 40 Curdling the emulsion.

This mass thus obtained whether homogenized or not, may be considered as made of a supporting medium of gelatin containing 45 particles of nitrocellulose carrying dye and oil, the oil comprising the emulgent and the amyl acetate solvent employed in the process. These particles of dyed nitrocellulose, containing oily material, will not mix 50 satisfactorily with other materials such as a silver bromid emulsion; hence I find it highly desirable to decrease the material, or to remove the larger portion of the amyl acetate solvent as well as the oil emulgent from 55 the nitrocellulose particles, and thereby obtain a mass of gelatin containing fairly pure semi solid particles of nitrocellulose intimately associated with a dyestuff. This may be accomplished by coagulating or curdling 60 the gelatin of the emulsion maintained as a sol or liquid by proper regulation of temperature, by adding it to an excess of electrolyte as, *e. g.*, a strong saline and preferably alkaline solution. For example, I may 65 use equal volumes of saturated sodium sul-

fate and sodium carbonate aqueous solutions, the carbonate rendering the solution alkaline. By this means a coagulum or curd of spongy consistency is obtained, this curd containing the dyed nitrocellulose particles dispersed 70 in gelatin, which has thus been converted from the hydrosol to the hydrogel condition.

#### Purification of curds and formation of sol.

The gelatin, when curdled or brought 75 into the gel condition, drags down or entrains globules of the nitrocellulose; but these nitrocellulose particles are substantially unaffected by the curdling operation, except in so far as the elimination of amyl acetate solvent tends to stabilize the particles and reduce their tendency to run together or be deëmulsified. By this method, the nitrocellulose particles are purified from a large part of the oil, since the latter remains largely in the solution, the gelatin and nitrocellulose being thrown down into a state comparable with a precipitated salt and separable from the oil and salt solution by filtration or other suitable methods. 80 While the main part of the oily matters, including the amyl acetate and the Turkey red oil remain suspended in the salt solution and can easily be separated from the curds, yet a portion of the saline solution and some 85 of the oil remain mechanically entrapped in the curds. These impurities may be removed by suitable methods, such as by pressure, or the curd may be removed from the saline bath, melted, filtered and then reset. 90 In any case, the curd or curdled emulsion is finally washed in a cold very dilute acid such as sulfuric acid to neutralize the alkalinity of the mass, and then in ice water, to remove the excess of neutral salts and oily 95 matters.

In order to put the material back into the sol condition, the curd or coagulum is melted in a water bath and if required its concentration is adjusted, to thin or thicken the 100 gel and form a uniform suspension by an addition of water or gelatin as is required. The mass is then filtered, if necessary, through felt or the like to remove any scum, if such be present, although it may 105 obviously be separated by any suitable method, such as skimming, straining, filtering, etc. This step in the process tends to homogenize the suspension or emulsion, since only the finer particles get through the 110 filter, depending, of course, upon the size of the filter openings.

There is thus obtained a uniform, stable emulsion or suspension, depending on the condition of the particles, of more or less 115 partially gelatinized nitrocellulose in gelatin, the particles of the mass being more or less permeated with dye, which is in a fixed relation with the nitrocellulose and will not wander or bleed. In other words, the dye in 120

the nitrocellulose particles is wash fast, although not necessarily light fast, as regards treatment with water and such other chemicals as are ordinarily used in photographic operations. The state of suspension or the size of the colloidal particles may be controlled by modifying the conditions of the emulsification, heat treatment before and after curdling, etc., it being possible to obtain an emulsion in which the suspension is grainless or colloidal in state or in which the dyed material is present in grains varying from fine to the coarser sizes. For example, the grain size may be increased by a continuation of the heat treatment during the melting operation after the gelatin has been curdled. Furthermore, the transparency of the mass may be controlled to a certain degree, since the fine grained emulsion is more transparent than the coarse grained. The processes of making this emulsion, as described, do not alter or affect materially the properties of gelatin of value in the photographic field, such as solubility in hot water and permeability to solutions of photographic chemicals, as well as its desirable qualities whereby it may serve as an elastic carrying and binding medium for silver salts.

#### 80      *Formation of color plate.*

Having thus prepared an emulsion of dyed nitrocellulose in gelatin, I may coat this emulsion by any suitable method on a transparent film or plate in any desired manner, as indicated in the illustrative examples shown in the accompanying drawing in which Figures 1 and 2 are sections of sensitive photographic elements to which a separate color layer is applied; Fig. 3 is a section of a photographic element in which the color and sensitive emulsions are incorporated in one layer; Fig. 4 a color screen with a color field extending over the entire surface; and Figs. 5 and 6, color screens in which the color or colors are applied in some design.

In the figures, A indicates the support made of any suitable material; B a uniformly applied color layer made in accordance with my invention and C a sensitive emulsion; BC indicates a layer in which the sensitive and color materials are in one layer; B' indicates a single layer applied in a design and B'' a multicolor layer applied in a design.

The emulsion made as above described may be applied either throughout the entire surface of the element as shown in Fig. 4 to serve as a ray filter or in separated areas involving a dot, line or other configuration as shown in section in Figs. 5 and 6 for use as a screen plate, or for various photographic purposes, where a colored medium can be used on a transparent or opaque support,

such as glass, film or paper. Similarly, the dyed emulsion may be undercoated, as in Fig. 1, or overcoated, as in Fig. 2, on a support beneath or over photographic material, such as a layer of silver salt emulsion, in any desired configuration or throughout the entire surface of the support. To produce, for example as in Fig. 2, a photographic plate combined with a green ray filter, a plate A suitably coated with a silver-salt gelatin emulsion C may have applied over the silver salt a layer of my emulsion B, which has been dyed by means of malachite green. It is also feasible to mix my dyed emulsion with a sensitive emulsion, such as silver bromid in gelatin, and so incorporate the dyed material in intimate association with the sensitive substance, and thereafter coat a photographic support A with the mixture BC, which may be utilized in the art of color photography for the production of color pictures.

Having thus described my invention, what I claim as new and desire to secure by Letters Patent is:

90

1. Photographic material comprising finely divided color particles insoluble in the ordinary photographic baths, dispersed throughout a carrying medium.

95

2. Colored photographic material comprising a colloidal medium, permeable to water and to photographic solutions carrying finely divided, colored, translucent particles dispersed therein.

100

3. Photographic material comprising an emulsion of translucent material containing a water fast, nonmigratory dye.

105

4. A photographic element comprising a support and a coating thereon of an emulsion of fast dyed particles in a water soluble colloidal medium, said particles being unaffected by photographic developing solutions.

110

5. A photographic element comprising a support and a colloidal mass containing finely divided translucent particles having intimately incorporated therewith a water insoluble color material, which will not migrate from the particles to the surrounding medium.

115

6. Photographic material comprising a colloidal medium, permeable to water and to photographic solutions carrying emulsified, oil free, colored translucent particles.

120

7. A photographic element comprising a support and a mono-color coating of an emulsion of translucent, mono-colored, oil free particles thereon.

125

8. A photographic element comprising a support and a coating of a colloidal magma incorporating therewith an emulsion of translucent particles and a color material which will not wander from said particles to the colloidal magma.

9. A photographic element comprising a

130

support and a translucent colloidal medium containing emulsified particles of translucent material carrying a water fast dye associated therewith, which will not wander therefrom into the colloidal medium.

10. A photographic element comprising a support and an emulsion in a carrier of gelatin of translucent material incorporating a dye, said material having a greater affinity for the dye than has the gelatin.

11. A photographic element comprising a support and a colloidal magma carrying a finely divided cellulose compound therein.

12. A photographic element comprising a support and a colloidal magma carrying emulsified nitrocellulose therein.

13. Photographic material comprising gelatin and emulsified nitrocellulose therein.

14. Photographic material comprising a supporting medium of gelatin carrying finely divided particles of dyed nitrocellulose.

15. Photographic material comprising a supporting medium of gelatin carrying emulsified particles of nitrocellulose having incorporated therewith a dye stuff.

16. A photographic element comprising a support and a coating of a supporting medium of gelatin carrying a mono-color dyed suspension of nitrocellulose.

17. A photographic element comprising a support and photographically sensitive material and an emulsion of color particles thereon.

18. A photographic element comprising a support carrying photographically sensitized material and a colloidal magma containing finely divided translucent color particles thereon.

19. A photographic element comprising a support, photographically sensitive material and a colloidal magma containing emulsified translucent material incorporating a water fast dye which will not wander to the magma.

20. A photographic element comprising a support, photographically sensitive material and a colloidal magma containing emulsified nitrocellulose particles.

21. A photographic element comprising a support, and photographically sensitive material and an emulsion of translucent particles of colored nitrocellulose in gelatin on said support.

22. A mono color photographic element comprising a support and photographically sensitive material and a mono-color emulsion of nitrocellulose and dye stuff in gelatin on said support.

23. The process of manufacturing photographic material comprising the steps of coloring a substance capable of being finely divided, and finely dividing the colored substance in a colloidal medium.

24. The process of making photographic

material comprising the step of emulsifying translucent color material in a colloidal solution.

25. The process of making photographic material comprising the steps of incorporating a water fast color in translucent material and emulsifying the same in an aqueous gelatin solution.

26. The process of making photographic material comprising the step of emulsifying a cellulose compound in a suspending medium.

27. The process of manufacturing a colored element comprising the steps of incorporating a dyestuff in a cellulose compound, and emulsifying a solution of said dyed compound in a colloidal medium.

28. The process of making photographic material comprising the step of emulsifying nitrocellulose in a colloidal medium.

29. The process of making photographic material comprising the steps of coloring nitrocellulose and emulsifying the colored material in gelatin.

30. The process of making photographic material comprising the steps of dissolving nitrocellulose in a solvent and adding color to the nitrocellulose and then emulsifying in an aqueous gelatin solution.

31. The process of making photographic material comprising the steps of dissolving nitrocellulose in amyl acetate and incorporating a color with the nitrocellulose and then emulsifying the colored nitrocellulose in an aqueous gelatin solution.

32. The process of making a photographic material comprising the steps of forming a solution of nitrocellulose, emulsifying the same in gelatin and purifying the emulsion.

33. The process of making photographic material comprising emulsifying colored nitrocellulose in an aqueous gelatin solution, and homogenizing the emulsion to obtain uniformly sized particles.

34. The process of forming a photographic element comprising emulsifying colored nitrocellulose in gelatin and coating a support therewith.

35. The process of preparing a colored photographic element comprising dissolving nitrocellulose in amyl acetate, incorporating a water fast dye with the nitrocellulose, emulsifying the same in an aqueous gelatin solution and coating a support with the colored emulsion of nitrocellulose in gelatin.

36. The process of making photographic material comprising the steps of dyeing nitrocellulose, agitating a solution of the nitrocellulose in amyl acetate in the presence of an emulgent and aqueous gelatin while maintaining the temperature above the melting point of the gelatin to form a solution and removing the amyl acetate and emulgent from the emulsion.

37. The process of making photographic

material comprising the steps of dissolving nitrocellulose in an oily solvent, incorporating color material therewith, emulsifying the solution in an aqueous gelatin solution, 5 curdling the emulsion to remove oily solvent therefrom and reforming the sol condition of the emulsion.

38. The process of making photographic material comprising the steps of forming a 10 solution of nitrocellulose in amyl acetate, emulsifying the same in an aqueous gelatin solution, changing the gelatin from the hydrosol to the hydrogel condition, removing amyl acetate therefrom and reforming the sol, to produce an emulsion of nitrocellulose in aqueous gelatin.

39. The process of making photographic material comprising dissolving nitrocellulose in amyl acetate, adding thereto an 20 alcoholic solution of a dye which has a molecular affinity for nitrocellulose and will not wander therefrom into gelatin or into the ordinary photographic solutions, emulsifying the dyed nitrocellulose in a colloidal 25 solution of gelatin, adding an electrolyte thereto to curdle the gelatin colloid to form a gel, removing the bulk of the amyl acetate solvent therefrom, and reforming the sol condition of the colloid, thereby obtaining 30 a colloidal mass of gelatin carrying finely divided colored particles of nitrocellulose dispersed therethrough.

40. The process of making a photographic element comprising the steps of coloring nitrocellulose with a dye which normally 35 tends to wander from gelatin into nitrocellulose, and dissolving the nitrocellulose in an oily solvent, then emulsifying the nitrocellulose in a colloidal medium, removing the oily solvent and purifying the emulsion 40 and coating said emulsion of dyed nitrocellulose in its colloidal carrying medium on a photographic element.

41. The process of making photographic material comprising the steps of incorporating 45 an alcoholic dye solution with nitrocellulose, emulsifying a solution of nitrocellulose in an aqueous gelatin solution by agitating in the presence of an emulgent to form a hydrosol, adding an electrolyte to the 50 hydrosol to form a gel containing suspended nitrocellulose, removing impurities therefrom, melting the gel to reform the hydrosol and adjusting the concentration by adding water or gelatin as required. 55

In testimony whereof, I have signed this specification in the presence of two witnesses this 22d day of May, 1917, at Rochester, N. Y.

SAMUEL E. SHEPPARD.

Witnesses:

FRED H. GARDNER,  
C. E. MARTIN.